

July 7, 1959

A. LORENZ

2,893,860

METHOD AND APPARATUS FOR CONTINUOUSLY DEGASSING MOLTEN  
METALS, PARTICULARLY STEEL, BY EVACUATION

Filed Aug. 5, 1957

6 Sheets-Sheet 1



Fig. 1

INVENTOR

ALBERT LORENZ

By *Christie, Parker & Hale*  
ATTORNEYS

July 7, 1959

A. LORENZ

2,893,860

METHOD AND APPARATUS FOR CONTINUOUSLY DEGASSING MOLTEN  
METALS, PARTICULARLY STEEL, BY EVACUATION

Filed Aug. 5, 1957

6 Sheets-Sheet 2



Fig. 2

INVENTOR

ALBERT LORENZ

BY *Christie, Parker & Hale*  
ATTORNEYS

July 7, 1959

A. LORENZ

2,893,860

METHOD AND APPARATUS FOR CONTINUOUSLY DEGASSING MOLTEN

METALS, PARTICULARLY STEEL, BY EVACUATION

Filed Aug. 5, 1957

6 Sheets-Sheet 3

Fig. 3



INVENTOR

ALBERT LORENZ

BY *Christie, Parker & Hale*  
ATTORNEYS

July 7, 1959

A. LORENZ

**2,893,860**

**A. LORENZ** 2,895,600  
METHOD AND APPARATUS FOR CONTINUOUSLY DEGASSING MOLTEN  
METALS, PARTICULARLY STEEL, BY EVACUATION

6 Sheets-Sheet 4

Fig. 4.



*INVENTOR*  
*ALBERT LORENZ*

BY  
*Christie, Parker & Hale*  
ATTORNEYS

July 7, 1959

A. LORENZ

**2,893,860**

**A. LORENZ** 2,03  
METHOD AND APPARATUS FOR CONTINUOUSLY DEGASSING MOLTEN  
METALS, PARTICULARLY STEEL, BY EVACUATION

6 Sheets-Sheet 5



၁၃၁

INVENTOR  
ALBERT LORENZ

BY  
Christie, Parker & Hale  
ATTORNEYS

July 7, 1959

A. LORENZ

**2,893,860**

A. LORENZ  
METHOD AND APPARATUS FOR CONTINUOUSLY DEGASSING MOLTEN  
METALS, PARTICULARLY STEEL, BY EVACUATION

6 Sheets-Sheet 6



६  
१९

INVENTOR  
ALBERT LORENZ

BY  
Christie, Parker & Hale  
ATTORNEYS

1

2,893,860

**METHOD AND APPARATUS FOR CONTINUOUSLY DEGASSING MOLTEN METALS, PARTICULARLY STEEL, BY EVACUATION**

Albert Lorenz, Hanau am Main, Germany, assignor to W. C. Heraeus G.m.b.H., Hanau am Main, Germany, a corporation of Germany

Application August 5, 1957, Serial No. 676,131

Claims priority, application Germany February 21, 1957

**4 Claims. (Cl. 75—49)**

The present invention relates to a new method of expelling gases from molten metals, especially steel, by passing the same through an evacuated chamber.

The basic concept of expelling or extracting undesirable gases from metals by subjecting the molten metal to the influence of a vacuum has been known for a long time. This has been done, for example, by agitating the molten metal in the crucible under a vacuum by inductive heating means for such a length of time until it was sufficiently degassed.

Another known method consists in removing the undesired gases from the molten metal, particularly steel, before it is cast and portion-by-portion while in the casting ladle. Such degasification is carried out in an evacuated chamber and the necessary movement of the molten metal through the vacuum chamber is produced solely by gravity either by a free fall of the metal or by the rise of the barometric level of the molten metal into the evacuated chamber produced by gravity. All of these known methods have a series of disadvantages which are primarily connected with their requirement that great quantities of molten metal have to be moved back and forth. Although, these disadvantages were fully realized, they have so far been regarded as unavoidable since the difficulties of including a degasification process into the mechanical casting operation as well as the technical difficulties of degassing large quantities of steel at high temperatures did not seem to permit any other solution.

It has also been proposed prior to this invention to cast large quantities of steel in one charge into a vacuum chamber. This, however, requires extensive modifications of the technical process and special apparatus of very large dimensions, as well as very sensitive parts which are easily damaged in the rough operation of a steel foundry. Although in the production of castings of rimmed steel the advantages of a degasification of the metal by means of a vacuum have already been realized, it has so far not been possible to carry out such methods except by very expensive means and procedures.

It is the principal object of the present invention to provide a very simple and inexpensive method of degassing molten metals, and especially steel, in a vacuum without incurring any of the above-mentioned disadvantages, and in a manner so as to permit a smooth and continuous operation by means of a very simple apparatus.

It is a further object of the present invention to provide a method of continuously expelling the undesirable gases from molten metals by conveying the metal continuously into and out of an evacuated degassing chamber.

Another object of the invention is to provide a method of this type wherein a continuous circulatory flow of the molten metal from its container through an evacuated chamber above said container and back into the container may be produced by the provision of very simple means which permit the metal flowing into the evacuated chamber to be maintained therein at a level different from the level of the metal flowing out of the chamber.

A further object of the present invention is to provide

2

a method of the mentioned type wherein the molten metal is conveyed into the evacuated degassing chamber by feeding a suitable gas or vapor into the metal.

Another object of the present invention is to provide a method of continuously degassing molten metals by passing the molten metal into a vacuum chamber and, after the metal has been degassed therein, by returning it to the main body of metal by centrifugal force.

A further object of the present invention is to provide very simple and inexpensive apparatus for carrying out the new method and for attaining the various advantages thereof.

The degasification method according to the present invention principally consists in passing the molten metal, for example, steel, continuously from its container along one path into an evacuated chamber, and in then returning it to the container along another path. The apparatus for thus circulating the molten metal may be of very simple design. For producing the forces required for such circulation, the new method relies particularly upon the liquid condition and the relatively high density of the molten metal. The new method possesses all the advantages of a continuous process and, although it avoids the necessity of moving or agitating large quantities of molten metal as required in the prior noncontinuous methods, it is still capable of degassing such large quantities of metal very efficiently and within a very short time.

While a successful performance of a degasification process according to all previous methods relied entirely on and at great expense upon the use of gravity, the continuous method according to the present invention in combination with a new apparatus for conveying or circulating the molten metal through a vacuum chamber permits such process for the first time to be carried out practically independently of such force. Since the degasification process according to the new method operates continuously, and the rate of flow of the molten metal through the vacuum chamber is quite fast, a very large quantity of metal may be efficiently degassed within a short time even though the quantity of molten metal actually passing at any time through the vacuum chamber might be very small. The application of a forced circulation as provided by the invention also allows considerable freedom in designing the apparatus required for an efficient degasification. Thus, for example, an apparatus according to the invention has been designed which may be applied successively to different parts of the body of molten metal in a casting ladle or other vessel so that nearly all parts of the metal will be reached by the apparatus and be passed successively through the vacuum chamber and thus be degassed.

When the molten metal before being degassed flows from the ladle or other vessel along an intake conduit upwardly into the vacuum chamber, the reduction of the density of the metal caused by the formation of gas bubbles therein will carry or drive it to a higher level than the level from which the degassed metal will flow back into the vessel along the return conduit. According to the invention, this process is started and preferably also subsequently assisted by injecting a material of considerably lower density, preferably a gas or vapor, into the molten metal while the latter flows upwardly toward the vacuum chamber. If this material consists of insoluble gases, the gas bubbles then forming within the molten metal will increase in size while rising toward and into the vacuum chamber. This material will then again easily separate from the molten metal within the vacuum chamber together with the undesired gases originally contained in the metal. By injecting such material, the medium density of the molten metal caused by its own gases which allows it to flow of its own accord into the vacuum chamber to be degassed therein will be still

further reduced so that the metal will reach a still higher level in the vacuum chamber relative to the normal barometric level, that is, the level of the degassed metal. The low density material will therefore act as a carrier and convey the molten metal continuously into the vacuum chamber and produce therein the mentioned difference in levels which, in turn, results in a continuous and very efficient degassification of the molten metal and also in a continuous circulation thereof from the ladle toward and through the vacuum chamber and back to the ladle.

If the circulating apparatus is designed so as to maintain the molten metal flowing into the vacuum chamber at a considerably higher level therein than the metal flowing out of the chamber, the entire contents of the container or ladle holding the main mass of molten metal will be gradually and continuously passed through the vacuum chamber and thus be thoroughly degassed therein either in the form of a thin layer or stream or in the form of small droplets.

If the molten metal itself has a high gas content, the gas bubbles forming in the metal of their own accord may be utilized for continuously conveying the metal into the vacuum chamber. In such a case, it will only be necessary to start the proper flow by an initial insertion of supplementary gas or, after such start, merely to assist the continued flow by feeding a small stream of such gas into the rising metal. Also, if the degassing operation has been interrupted or the automatic formation of bubbles of the gases inherent in the rising metal diminishes, it may again become necessary to feed the extra gas either temporarily or continuously into the molten metal.

The present invention may also be modified by applying a circulating apparatus which assists in the discharge of the degassed metal from the vacuum chamber. In such event, the relatively high density of the molten metal itself may be utilized to considerable advantage for producing a centrifugal force for conveying the metal. Such centrifugal force may easily be made of sufficient size even though the necessary rotating parts of the apparatus are of small diameters and are driven at low speeds.

If the means for conveying the molten metal are furthermore applied to that part of the circuit where the degassed metal is returned to its container and not to that part where the metal before being degassed is conducted into the vacuum chamber, the amount of metal conveyed and the resistance to the flow thereof within such circuit may be controlled so that the level of the returning molten metal in the vacuum chamber will be lower than the level which would correspond to the difference in pressure between the outer atmosphere and that within the vacuum chamber.

The degassification apparatus according to the invention therefore essentially consists of a vacuum chamber which is disposed above the container holding the molten metal and is connected thereto by two separate conduits; and a mechanism for conveying the metal continuously from the vacuum chamber back into the container. Due to such forced circulation, the apparatus itself may be made of a relatively small size. This, in turn, renders the generation of the centrifugal forces utilized for effecting the circulation a very simple matter. These forces may, for example, be generated by securing the return conduit of the molten metal to the bottom of the vacuum chamber and coaxially thereto, by providing the lower end of this conduit with a disklike member of a larger diameter, by immersing this lower end of the return conduit, as well as the intake conduit, which extends within the return conduit and coaxially thereto into the molten metal within the container, and by rotating the vacuum chamber together with the return conduit within the molten metal. The degassed metal returning from the vacuum chamber and arriving at the

disklike member at the lower end of the return conduit will then be expelled therefrom into the surrounding metal in the container by the centrifugal force produced by the rotation.

The circulating mechanism therefore consists of two parts, a mechanical part and a functional part, the mechanical part consisting of the disklike end of the return conduit within the container holding the body of molten metal, and the functional part consisting of the rotation of the vacuum chamber together with the return conduit. The inter-action of these two parts results in a highly effective and simple circulating mechanism.

Further objects, features, and advantages of the present invention will be apparent from the following detailed description thereof, particularly when read with reference to the accompanying drawings, in which—

Fig. 1 shows, largely in cross section, an apparatus according to the invention in which the molten metal is conveyed into the vacuum chamber by means of a supplementary gas fed into the metal;

Fig. 2 shows a similar view of a modification of the apparatus illustrated in Fig. 1;

Fig. 3 shows a similar view of another apparatus according to the invention in which the molten metal is returned from the vacuum chamber into the container by means of centrifugal force;

Fig. 4 shows partly in cross section a detail view of a modified portion of the apparatus according to Fig. 3;

Fig. 5 shows, partly diagrammatically, a general view of an entire degassification plant according to the invention during its operation; while

Fig. 6 shows a view similar to Fig. 5 but with the degassification apparatus in the inoperative position.

Referring to the drawings, and first particularly to Fig. 1, a vacuum pump 1 is connected to a vacuum chamber 2 by a pump line 3. Vacuum chamber 2 is formed by a tank 4 having a bottom 5 to which short pipes 6 and 7 are connected which are adapted to be partly immersed into the molten metal 8 within a container or casting ladle 9. This ladle 9 has a lining 10 and a tap-hole 11 which is adapted to be closed from above by means of a plug 12.

After the apparatus is lowered into ladle 9 so that the lower ends of pipes 6 and 7 are immersed into the molten metal 8 to a point below the surface 13 thereof, chamber 2 is evacuated whereby the molten metal rises within pipes 6 and 7 to the barometric level  $h_a$ .

A pipe line 14 is adapted to be inserted into the molten metal 8 in ladle 9 so that its end 15 is disposed at a point closely underneath or within the lower end of pipe 6. Pipe line 14 is connected to a source of supply of a suitable gas, not shown, and adapted to conduct such gas into the molten metal in pipe 6. The gas bubbles will then rise in pipe 6 and, in the course of their ascent, they will increase in size. They have the tendency to take along the molten metal in pipe 6 into vacuum chamber 2 in the direction as shown by the arrow 17.

These gas bubbles reduce the density of the molten metal in pipe 6, thereby causing the metal to rise to a higher level than the barometric level  $h_a$  of the solid metal column in pipe 7. The metal thus enters from pipe 6 into vacuum chamber 2 in which the added gas is separated from the metal, while the undesired gases contained therein are likewise expelled. The molten metal then flows in the direction shown by arrow 18 toward and into the return pipe 7 and then back to the main body of metal 18 in ladle 9. In order to prevent the molten metal from splashing too far upwardly into chamber 2, a stationary deflecting plate 20 may be provided within chamber 2 at a certain height above the mouth of pipe 6.

In the embodiment of the invention as shown in Fig. 1, pipe line 14, 15 through which the conveying gas is supplied into the molten metal in the intake pipe 6 forms an independent element separate from vacuum tank 4

and pipes 6 and 7. This pipe line is adapted to be removed from ladle 9 after the flow of molten metal in the direction of arrows 16, 17, 18, and 19 has been started by the added gas, provided the molten metal itself contains sufficient gas or still contains the same to maintain the flow after such start or after the degasification has been carried out for a certain length of time. When the gas content of the molten metal in ladle 9 has been diminished to such an extent that the continued automatic circulation without the addition of supplementary gas will be interrupted or is soon liable to cease, pipe line 14, 15 is reinserted into pipe 6 to start the flow or to assist it by a further supply of conveying gas.

Fig. 2 illustrates a modification of the apparatus shown in Fig. 1. In this case, the gas line 21, 22 is secured by a vacuum-tight connection to vacuum tank 4 and extends centrally from above through the intake pipe 6, terminating at or near the lower end thereof.

The added conveying gases may consist of any suitable inert gases, for example, argon, which are not soluble or only slightly soluble in the molten metal. However, other gases such as those contained to some extent in the molten metal itself, for example, nitrogen and carbon monoxide, may also be used with equal results since they are separated in any event from the molten metal within the vacuum chamber.

In certain cases it is also possible to combine the introduction of gas for conveying the molten metal into the vacuum chamber with additional purposes. Thus, for example, if iron or steel are to be degassed, the introduction of oxygen into the molten metal will assist in carrying out the necessary refining process thereof.

The vacuum chamber may also be provided with additional means for effecting or facilitating the separation of the gases from the metal which usually splashes around in the chamber in the form of large drops or jets. A simple form of such means may consist of the deflecting plate 20 as shown in Figs. 1 and 2. However, these separating means within the vacuum chamber may also consist of moving elements, for example, a revolving plate or the like.

However, the important feature of the method as above described is that it does not require any movable parts, and particularly no rotary movement of the apparatus, but that it only relies upon the buoyancy of a mixture of gas and molten metal for conveying the metal into and through the vacuum chamber. This method is therefore of greatest simplicity and may be carried out by means of a very simple and inexpensive apparatus.

Fig. 3 illustrates a modification of the invention which relies upon the same basic principle as the embodiments shown in Figs. 1 and 2, namely, of effecting a constant circulation of the molten metal through the vacuum chamber and of thus attaining a continuous gasification of the metal by producing a difference in density of the molten metal within the intake and return pipes of the vacuum chamber. However, instead of reducing the density of the metal within the intake pipe so as to raise the intake level of the metal relative to the normal barometric level  $h_a$ , that is, the level within the return pipe, by injecting an extra gas into the metal within the intake pipe, the modification according to Fig. 3 relies upon the principle of lowering the level of the surface of the degassed metal within the vacuum chamber relative to the normal barometric level  $h_a$  by means of centrifugal force.

The apparatus for carrying out this method, as illustrated in Fig. 3, consists of a vacuum pump 101 which is connected by a pipe 102 to a dust separator 103 which, in turn, is connected by a pipe 104 to a stationary container 105 with a cover 106. On its inner wall, container 105 carries suitable bearing means 107 for rotatably supporting a container 108 which forms the main vacuum chamber. A leakage of outside air into containers 105

and 108 is prevented by providing sealing rings 109 and 110, as well as an annular chamber 111 between the outer wall surface of the reduced neck portion 112 of container 108 and the inner surface of container 105, and by connecting such chamber 111 to vacuum pump 101 by means of a pipe 113 so that vacuum chamber 108 will be continuously evacuated.

Vacuum chamber 108 and its upper tubular end 112 may be rotated by a motor 114 through reduction gears 115, for example, in the direction as shown by arrow 116.

The walls of vacuum chamber 108 may also have a lining (not shown). The substantially parabolical bottom portion 117 of container 108 has a tubular 118 portion secured thereto which may either be a solid pipe or be likewise lined. This tubular portion 118 carries coaxially thereto an inner pipe 119 by means of spacing members 120. The upper end of pipe 119 extends for a certain distance into container 108.

The lower ends of the coaxial pipes 118 and 119 extend into a container or casting ladle 121 and are immersed into the molten metal 122 for a certain distance below the surface 123 thereof. Ladle 121 is provided with a lining 124 and a taphole 125 which may be closed from above by a plug 126. Below the surface 123 of the molten metal in ladle 121, the outer or return pipe 118 terminates in an annular disklike member 127, thus forming an annular passage between disks 127 and 128 which communicates with the return passage in pipe 118. The two disks 127 and 128 may be further secured to each other in the proper spaced relation by spacing members 129 which divide the annular passage into a plurality of separate channels which improve the return flow of molten metal into the main body of metal 122 in ladle 121 as subsequently described.

35 The lower end of the apparatus consisting according to Fig. 3 of the coaxial pipes 118 and 119, disks 127 and 128, and the spacing and supporting members 120 and 129 may also be made of highly refractory ceramic material, as illustrated in Fig. 4. The reduced lower end

40 130 of vacuum tank 108 which may have a lining 131 merges into the ceramic part 132, and these two parts are preferably disconnectable from each other in a suitable manner, not shown. The ceramic part 132 consists of the central intake channel 133 and a plurality of vertical 45 return channels 134 surrounding the intake channel 133 and terminating at the lower ends in radially extending outlet channels 135 having outlet openings 136. When the vacuum tank 108 is rotated, the molten metal contained in the radial channels 135 produces the centrifugal 50 force which effects the continuous movement of the metal from vacuum chamber 108 into the main body of metal 122 in ladle 121.

For carrying out the method according to the invention, the degasification apparatus is lowered into the molten metal 122 in ladle 121 substantially to the position as shown in Fig. 3 and is then evacuated by pump 101. The metal will then rise into vacuum chamber 108 until it reaches a level of a height  $h_a$  which corresponds to the barometric pressure attained at the respective degree of evacuation which for steel amounts to a maximum of approximately 140 cm. Motor 114 is then switched on so as to rotate vacuum tank 108 and the coaxial pipes 118 and 119 with disks 127 and 128 thereon.

The revolving disks 127 and 128 with the spacing members 129 transmit their movement to the intermediate amount of molten metal which is then thrown outwardly in the direction shown by arrows 137. The velocity of the throw depends upon the speed of revolution and the diameter of disks 127 and 128 since these two values aside from the density of the molten metal determine the power of the centrifugal force. For practical purposes, the disks are preferably made of a diameter of approximately 50 cm. and the speed is made 1 to 3 revolutions per second.

75 The amount of molten metal thrown out between disks

**127** and **128** or outlet openings **136**, as shown in Fig. 4, respectively, is continuously replenished by the flow of metal from vacuum chamber **108** through pipes **118** and **119** in the direction shown by arrows **138** and **139**. Since the barometric pressure allows the molten metal to penetrate into chamber **108** up to the level  $h_a$ , the metal will continue to flow into and through intake pipe **119** in the direction of arrows **138** since within this central pipe it will be only very slightly affected by the centrifugal force produced by the rotation and acting in direction **137** vertically to the direction of flow **138-139**.

If the speed of rotation, the diameter of disks **127** and **128**, and the resistance to the flow within intake pipe **119** are all made of the proper size, the level of the molten metal within vacuum chamber **108** will be lowered a substantial extent below the normal barometric level  $h_a$ , for example, to the level  $h_b$ . Thus, there will no longer be a uniform surface which connects the inner intake flow with the outer return flow of the metal. This has the great advantage that the metal will flow very quickly through chamber **108** and result in a free flow therein which insures a very efficient degasification of the metal.

Since the molten steel rising through the inner pipe **119** contains considerable quantities of gases which even under standard conditions may amount to a multiple of the volume in metal, the enclosed gases will normally urge toward the surface within the vacuum chamber, thereby taking along the metal. Since the pressure upon the metal progressively decreases as the metal rises to a higher level within the intake pipe **119**, the enclosed gases will separate with increasing intensity. This results in the formation of gas bubbles which more and more increase in volume as they are reaching a progressively higher level, thus pushing the metal above them into the vacuum chamber. These gas bubbles when finally bursting within the vacuum chamber also finely distribute and scatter the metal into small particles. The molten metal will thus attain a very large surface area within the vacuum chamber, be more extensively subjected to the action of the vacuum, and be thoroughly degassed. Since, on the other hand, the metal in return pipe **108** is fully degassed and, except for its return flow, perfectly quiet, the difference between the height of the intake and return levels will be very considerable.

The mentioned fine and thorough distribution of the molten metal within vacuum chamber **108** may be further increased by making the intake pipe **119** of a height so as to extend above the level  $h_b$  but not to reach the barometric level  $h_a$ . The metal will thus be freely ejected at a high velocity from the mouth of pipe **119** in the upward direction and be more thoroughly exposed to the vacuum by its fountainlike flow within chamber **108**. In order to prevent the molten metal from being shot upwardly into the upper stationary tank **105** and from entering into the pump line **104**, a deflecting plate **140** which is capable of resisting the high temperatures of the molten metal is mounted within chamber **108**. The upper end of intake pipe **119** may also have an annular projecting flange **141** or be provided with slots or other suitable means in order to increase its distributing action upon the molten metal.

Fig. 5 diagrammatically illustrates the entire degasification plant according to the invention with all of its essential parts. The pump unit **201** is connected by a movable vacuum pipe **202** with articulated joints **203** to the dust separator **204** which, in turn, is connected by means of a suction pipe **205**, which also serves as a supporting beam, to a head **206** similar to member **100** in Fig. 3 which supports the rotary vacuum tank **207** and is connected thereto by rotary bearing and sealing means **208**. A motor **209** is connected by reduction gears or a chain drive **210** to vacuum chamber **207** to rotate the same. Chamber **207** carries at its lower part the two coaxial pipes **211** and **212** which terminate in a disklike member **213** with openings **214** which communicate with the space intermediate pipes **211** and **212**.

and thus with the inside of chamber **207**. The lower end of this apparatus with the disklike member **213** thereon is immersed from above into the molten metal **215** within a casting ladle **216**.

Suction pipe **205** which also serves as a supporting beam for carrying vacuum chamber **207** and all the parts connected thereto is pivotally mounted on an upright **217** by means of a pair of bearing brackets **218** and a pivot shaft **219**. Upright **217** is vertically slidable within a cylinder **220** and adapted to be raised and lowered by hydraulic means within cylinder **220**. A guard plate or partition **221** mounted on the upper end of upright **217** protects the various elements at the right of ladle **216** and vacuum tank **207** as well as the operator from the heat radiated from the ladle and tank and any possible molten metal particles spattering out of ladle **216**.

Cylinder **220** is mounted on a platform **222** which also supports a pair of beams **223** at the right side of upright **219** which are connected at the upper end and above suction pipe **205** by a crossbar **224**. Platform **222** further supports a hydraulic pump unit **225** for raising and lowering upright **217** with suction pipe **205** and all of the elements connected thereto and for thereby also pivoting suction pipe **205** and all of these elements about the pivot **209**. A control panel **226** with an operator's stand is also mounted on platform **222** which is provided with wheels **227** which may be driven by a motor **228** to move the entire apparatus on rails **229** relative to ladle **216**.

Fig. 6 finally illustrates a degasification plant with a vacuum tank similar to that shown in Fig. 2 and an operating mechanism similar to that shown in Fig. 5 but in a position prior to the degassing operation. The upright **217** is then hydraulically elevated, whereby the suction pipe **205** bears against crossbar **224** and is pivoted about shaft **219**. Vacuum tank **230** is thus likewise raised and pivoted. After platform **222** is moved to the proper position relative to the casting ladle **216**, upright **217** is lowered, whereby vacuum tank **230** is pivoted to its vertical position and its lower end immersed into the molten metal in ladle **216**. Vacuum tank **230** is mounted on suction pipe **205** and consists of the main chamber **231** with an intake pipe **232** and a return pipe **233** at the lower end of chamber **231** and a bottom **234** of chamber **231** which inclines downwardly from pipe **232** toward pipe **233** to facilitate the return flow. A feed pipe **235** which is connected to a supply of a suitable gas (not shown) extends through chamber **231** and centrally through intake pipe **232** to a point near the lower end thereof.

A detailed description of the operation of vacuum chambers **207** and **231** as shown in Figs. 5 and 6, respectively, has already been given above and therefore needs not be repeated.

Although my invention has been illustrated and described with reference to the preferred embodiments thereof, I wish to have it understood that it is in no way limited to such particular embodiments or to the details thereof, but is capable of numerous modifications within the scope of the appended claims. The important concept of the present invention as defined by these claims is to provide a method and a suitable apparatus for continuously conveying the molten metal into a vacuum chamber to be degassed therein and then to return it to its container by producing a noticeable difference in the level of the molten metal fed into the vacuum chamber and the level of the molten metal within the chamber which is ready to be removed therefrom. The two different methods as described above may also be combined with each other in that a supplementary conveying gas may be fed into the intake pipe **118**, **133**, or **212**, as shown in Figs. 3, 4, or 5, respectively. The particular means for carrying out the conveying movement of the molten metal into and from the vacuum chamber may

also be of a different type and design than shown in the drawings and above described. Thus, for example, it is possible to use an electro-magnetic pump which moves the molten metal by means of an electric current within a magnetic field. The apparatus according to the invention also have the great advantage that they may be made of a mobile construction and be easily moved from one casting ladle to another, and that they are movable and pivotable and thus capable of reaching almost any part of the body of molten metal within a casting ladle.

Having thus fully disclosed my invention, what I claim as new is:

1. An apparatus for continuously degassing molten metals comprising a container adapted to hold a body of molten metal, a chamber disposed above said container and having an intake conduit and a return conduit at the lower end thereof adapted to be partly immersed into said body, a substantially circular outlet member on the lower end of said return conduit and coaxial thereto, said outlet member having a diameter larger than the diameter of said return conduit and having a plurality of substantially radially extending outlet channels therein, means for continuously evacuating said chamber when said conduits are immersed in said body, and means for rotating at least said outlet member, whereby when said outlet member is rotated within said body of metal, the molten metal contained within said channels will be subjected to a centrifugal force and be ejected from said channels into said metal body, thereby producing a circulation of said molten metal from said body through said intake conduit into said chamber to be degassed therein and back through said return conduit and said outlet member into said metal body.

2. An apparatus as defined in claim 1, further comprising means for injecting a gaseous material into said intake conduit near the lower end thereof.

3. An apparatus for continuously degassing molten metals comprising a container adapted to hold a body of molten metal, a chamber disposed above said container and having an inner intake conduit and an outer return conduit coaxially with said chamber within each other and secured to the bottom of said chamber, a pair of annular disklike members of a larger diameter than

5  
10

said outlet conduit and coaxial with said conduits, one of said members being secured to said intake conduit near the lower end thereof and the other member being secured to the lower end of said outlet conduit, means for continuously evacuating said chamber when said disklike members on said conduits are immersed in said body, and means for rotating said chamber with said conduits and members whereby when said disklike members are immersed in said body and when said chamber with said conduits and members are rotated, the rotation of the molten metal between said members produces a centrifugal force for ejecting the molten metal from said return conduit into said metal body and thereby produces a circulation of said metal from said body through said intake conduit into said chamber to be degassed therein and back through said return conduit into said metal body.

4. A method of continuously degassing molten metals comprising the steps of continuously evacuating a chamber disposed above a container and directly communicating with a body of molten metal in said container by a pair of conduits disposed coaxially around each other, connected to the bottom of said chamber and partly immersed into said body of metal, conducting the metal through the inner conduit into said chamber to be degassed therein, and rotating at least the outer conduit about its axis so that the degassed metal within said outer conduit will be subjected to a centrifugal force and by the action of said force be continuously withdrawn from said chamber and ejected into said body of metal, wherein said centrifugal force is produced by the lower end portion of the rotating outer conduit which is submerged in said body of molten metal and separates the metal within said end portion into a plurality of substantially radially extending bodies and then passes the metal to a plurality of streams into said main body of molten metal.

References Cited in the file of this patent

UNITED STATES PATENTS

291,223 Pielsticker et al. ----- Jan. 1, 1884  
1,921,060 Williams ----- Aug. 8, 1933

UNITED STATES PATENT OFFICE  
CERTIFICATE OF CORRECTION

Patent No. 2,893,860

July 7, 1959

Albert Lorenz

It is hereby certified that error appears in the printed specification of the above numbered patent requiring correction and that the said Letters Patent should read as corrected below.

Column 6, line 17, for "cer--" read -- certain --; line 22, for "Laddle" read -- Ladle --; line 60, "exacuation" read -- evacuation --.

Signed and sealed this 29th day of December 1959.

(SEAL)  
Attest:

KARL H. AXLINE  
Attesting Officer

ROBERT C. WATSON  
Commissioner of Patents